

F. LAIST.

ROASTING FURNACE.

APPLICATION FILED DEC. 23, 1912.

1,070,490.

Patented Aug. 19, 1913.

4 SHEETS-SHEET 1.

FIG. I.



WITNESSES:

Harry A. Barnes  
J. C. Martin

INVENTOR.  
Frederick Laist.

BY *Emil Stares*  
ATTORNEY.

1,070,490.

F. LAIST.  
ROASTING FURNACE.  
APPLICATION FILED DEC. 23, 1912.

Patented Aug. 19, 1913.

4 SHEETS-SHEET 2.



**WITNESSES:**

Harry A. Benney  
Jacomich

INVENTOR.  
Frederick Laist.

BY Amelia  
ATTORNEY.

F. LAIST.  
ROASTING FURNACE.  
APPLICATION FILED DEC. 23, 1912.

1,070,490.

Patented Aug. 19, 1913.

4 SHEETS—SHEET 3.



WITNESSES:

Harry A. Beiner

Joamichel

INVENTOR.  
Frederick Laist.

BY

Ant. Stora

ATTORNEY.

F. LAIST.  
ROASTING FURNACE.  
APPLICATION FILED DEC. 23, 1912.

1,070,490.

Patented Aug. 19, 1913.

4 SHEETS-SHEET 4.



WITNESSES:

Harry A. Beimes  
Josephine

INVENTOR.  
Frederick Laist.

BY Curtis L. Bixler  
ATTORNEY.

## UNITED STATES PATENT OFFICE.

FREDERICK LAIST, OF ANACONDA, MONTANA.

## ROASTING-FURNACE.

1,070,490.

Specification of Letters Patent. Patented Aug. 19, 1913.

Application filed December 23, 1912. Serial No. 738,249.

*To all whom it may concern:*

Be it known that I, FREDERICK LAIST, a citizen of the United States, residing at Anaconda, in the county of Deerlodge and State of Montana, have invented certain new and useful improvements in Roasting-Furnaces, of which the following is a full, clear, and exact description, reference being had to the accompanying drawings, forming 10 a part hereof.

My invention has relation to improvements in roasting furnaces; and it consists in the novel details of construction more fully set forth in the specification and 15 pointed out in the claims.

In the drawings, Figure 1 is a combined elevation and middle vertical section of the furnace, the section being taken through one of the fire-boxes; Fig. 2 is a top plan, parts 20 being broken away; Fig. 3 is an enlarged vertical sectional detail of the upper hearth or floor, with parts of the ore-feed mechanism in elevation; Fig. 4 is a horizontal section on the line 4—4 of Fig. 1 taken above 25 the rabble-arms in the direct-fired hearth, parts being broken away; Fig. 5 is an enlarged vertical section on the curved line 5—5 of Fig. 4 showing the detailed construction of the feed-hopper leading from 30 the third to the fourth hearth; Fig. 6 is a combined elevational and sectional detail showing the rabble-shaft and the sand-seal which is interposed between the third and 35 fourth hearths; and Fig. 7 is a diagrammatic plan showing the relative position of the drop holes leading from the second to the third hearth, and the discharge openings from the fire-box leading into the third hearth.

40 The present invention is directed to improvements in a type of roasting furnace known as the McDongal, the objects in view being to make this type serviceable for roasting and chloridizing ores, particularly 45 low grade ores, in order that their metal content may be readily brought into solution by the action of an acid solvent (or leaching solution). Where copper ores containing silver are treated, the solvent employed is sulfuric acid and salt dissolved in water in the proportions of about five per cent. by weight of acid and from five to fifteen per cent. of common salt.

50 A further object of the invention is to construct a furnace in which the loss of copper fumes (in the chloridizing process) will

be almost entirely overcome; one in which the chloridation may be effected without the application of external heat, the heat of the calcines delivered from the roasting hearths 60 to the chloridizing hearths being sufficient for that purpose; one in which overheating of the charge is prevented, thereby avoiding the formation of compounds (notably ferrite copper) which are insoluble in 65 the leaching solution; one which shall be properly insulated against the loss of internal heat; one in which the charge on the successive hearths is rabbled only at such intervals as the character and condition of the 70 material demands; and one possessing further and other features whose advantages will be better apparent from a detailed description of the invention which is as follows:

75 Referring to the drawings, F represents the furnace (extending partly above and partly below the floor-line L), and a, b, c, d, e, f, the several superimposed hearths in which the material is treated (the present 80 being a six-hearth multiple-hearth furnace), the material dropping from the upper hearths successively through the several hearths until it is delivered into the discharge hopper C, the hearths being provided 85 with the central and marginal openings or drop-holes o, o', for the passage of the material. Passing centrally through the hearths is the rotatable hollow rabble-shaft 1 from 90 which radiate the series of hollow rabble or stirrer arms 2 extending into the several hearths and carrying rakes 3, by which the material is successively fed from one hearth to the hearth immediately beneath it, the shaft and arms being provided with water-circulating cooling pipes P, P', as fully understood in the art. In the present case the rabble mechanism (shaft, hollow arms, and rakes) is driven by a worm 4 engaging a worm-gear 5 on the upper end of the rabble-shaft. On the quill 6 carrying the worm 4 is a sprocket 7 from which leads a chain 8 passing over a sprocket 7' and operating a shaft 9 on which are disposed sprocket-wheels 10, 10', 10'', 10''' of various diameters corresponding, but set in reverse order to, a similar set of sprocket wheels 11, 11', 11'', 11''', on the parallel shaft 12 of the feed-screw 13 in the feed hopper H. A loose chain 14 which can be shifted to any pair of sprockets drives the feed-screw, thus giving four speeds. The feed can also be

adjusted by means of a sliding plate 15 positioned immediately over the feed-screw and actuated by a pinion 16 engaging a rack 17 on said plate (Figs. 2, 3). The quill carrying the worm 4 and the sprocket 7 can be clutched to the main-shaft 18 running over a row of furnaces, by means of a clutch K whereby the rabble mechanism and feed can be started or stopped simultaneously. The clutch-shifter is not here shown as that is well understood in the art.

The present is a direct-fired furnace being provided with two diametrically opposite fire-boxes B, burning coal (though coal-dust, oil, or gas may be substituted), each fire-box having a shaking grate G, an ash latinder A, and a checker-work arch W, and discharging its gases and combustion products into the hearth c or hearth number 15 three counting from the top. This hearth is considerably deeper than any of the remaining hearths there being left a clearance of from ten to twelve inches between the upper surface of the rabble-arms in said hearth 20 and the roof of the hearth, the gases from the fire-boxes discharging into said hearth through the openings O which are located above the rabble arms and contiguous to the outer edge of said roof. As seen best in 25 Figs. 1 and 7, the drop holes o' of the second hearth (b) (always counting from the top) discharge the material onto the floor of the third hearth c, the position of these particular marginal drop-holes relatively to the 30 discharge openings O being shown to best advantage in Fig. 7. In hearth c the roasting-ore is moving away from the circumference toward the center drop holes (special center drop holes being provided for this 35 hearth as presently to be fully described). The ore is likewise moving away from the fire-boxes, this being an important feature of my invention for the following reason:—

In any direct-fired furnace used for roasting 40 copper ore for leaching purposes, it is very important to avoid overheating any of the ore since to do so causes a portion of the copper contents to become insoluble in the leaching solution, owing to the formation of 45 ferrite copper. The temperature on the second floor or hearth b is by measurement approximately 540 degrees Fahr. about two feet radially from the point where the ore drops onto the third floor (c). Before the 50 formation of "insoluble copper" (ferrite copper) becomes serious a temperature of at least 1100 degrees Fahr. must be exceeded, so that the quantity of insoluble copper on this floor (b) is negligible and it makes no 55 difference what the relative movement of the ore and flame thereover may be. On the third floor (c) however, conditions are different. Here we have a temperature of 60 1280 degrees Fahr. about two feet from the 65 furnace walls and about midway between

the drop-holes (from hearth b) and the gas discharge or fire-box openings O, the temperature being even higher closer to the said openings. The ore dropping from the second floor (b) has a temperature of about 500 degrees Fahr.; and were it permitted to move toward this region or zone of high temperature, the tendency would be for portions of the ore to become overheated and rendered insoluble as above pointed out. 75 This overheating will obviously be much reduced by having the comparatively cool ore entering said heated region or zone, moved continually toward a region of less heat or lower temperature, that is to say toward the center of the hearth. Accordingly, in a multiple hearth furnace roasting ore for leaching by direct firing, it is essential that the direct-fired hearth shall be one in which the ore is moved toward the center or away 80 from the zone of high temperature prevailing at the point of discharge of the gases from the fire-box into the hearth. In my present construction therefore, the fire-box is allowed to discharge into the third hearth 85 c in which the rakes move the ore from the circumference toward the center. It is also important, in order to minimize the formation of insoluble or ferrite copper, and to prevent the destruction and deterioration of 90 the rabble arms and rakes in this hearth (c) that the openings O from the fire boxes shall be immediately under the roof of the third hearth, and that this roof shall be so high above the rabble arms that the flame will 100 clear the arms and play between the roof and said arms (Fig. 1). It is for this reason that a clearance of from ten to twelve inches is left between the upper surface of the rabble arms and the roof of the third 105 hearth, the rabble arms being thus brought out of range of the gases from the openings O.

In general, there are two types of roasts made use of for rendering soluble in dilute acids the copper contents of sulfid ores, to-wit:—(1) an oxidizing or sulfating roast, and (2) a chloridizing roast. My present furnace combines these two types, the ore being oxidized on the three upper hearths 110 or floors a, b, c, and chloridized on the three bottom floors d, e, f, the temperature of the charge being raised sufficiently high on the oxidizing floors to permit of a rapid chloridizing action on the lower floors. The furnace walls of the three bottom floors are insulated against heat loss by radiation by a layer of asbestos 115 or equivalent material, or by making the walls sufficiently thick to prevent loss of heat, or by means of an air 120 space, the bottom floor being likewise properly insulated. The insulation referred to is important since the lower floors (d, e, f) in which the chloridation is taking place 125 are heated solely by the heat of the calcine 130

discharged from the upper or oxidizing hearths or floors and which works down through said lower floors. The salt entering into the chloridizing reaction is fed to the fourth floor (*d*) in proper quantities through the doors *D*, said salt chloridizing all the silver present (usually a mixture of  $\text{Ag}$ ,  $\text{Ag}_2\text{S}$ ,  $\text{Ag}_2\text{SO}_4$  as a result of the oxidizing roast) as well as that portion of the copper which may have escaped conversion into oxid on the upper floors. This portion is generally a copper sulfate and is converted into chlorid as per following reaction:—



A portion of the copper oxid may however, also undergo chloridation as obvious from the following reaction:—



the aim being to always add sufficient salt to chloridize all the silver and that portion of the copper not converted into oxid in the 25 oxidizing roast. The consequence is that the composition of the final calcine which is to be leached, is substantially a mixture of copper oxid, copper chlorid, and silver chlorid, any iron present being converted 30 into an oxid by the heat and oxygen present, thus—



The leaching solution employed is water 35 containing about five per cent. by weight of sulfuric acid and ten per cent. by weight of common salt, such solution readily dissolving the several components of the calcine referred to (the gangue or sand of course, 40 being insoluble).

In all chloridizing roasting, a certain percentage of the copper (usually as chlorid) volatilizes, and to save these fumes it becomes necessary to condense the same in absorption towers. In my present furnace 45 wherein the chloridation takes place in the three lower hearths, it becomes necessary therefore to provide some means for preventing the escape of these fumes from the chloridizing hearths (*d*, *e*, *f*) into the oxidizing hearths (*a*, *b*, *c*), while at the same time permitting free passage of the calcine from the third (*c*) to the fourth (*d*) hearth. If the fumes from the lower hearths were 55 allowed to escape to the upper hearths, they would suffer too great a dilution with the fire-gases, a consequence avoided herein, by the provision of specially constructed hoppers which take the place of the central drop holes *o* above referred to. What would otherwise substantially correspond to a central drop hole *o* between the third and fourth hearths (*c*, *d*) is closed by a sand-seal 60 20, the seal being formed by an annular 65 trough 21 forming the upper terminal of a

sleeve *w* inserted through and forming a lining for the central opening *o* in the floor of the hearth *c*, and a flanged disk 22 snugly passed over the shaft 1 and with its flange or rim dipping under the surface of the sand in the trough and thus completing the seal. The seal 20 thus prevents escape of fumes from the fourth to the third hearth, the calcine being however free to drop from the third to the fourth hearth through the special hoppers 23, 23, disposed on the floor of the third hearth (*c*) at points diametrically opposite one another and in proximity to the sand seal 20. The passage-way of the hopper corresponds to a section of the space 70 between the walls of two cylinders concentric with the axis of the rabble-shaft and separated or spaced slightly apart, the sides of the hopper tapering downward and the bottom thereof being provided with a discharge spout 23' the outlet of which is made as small as is consistent with the free and unobstructed passage of the calcine therethrough (Fig. 5). As just stated, the degree of separation between the opposing walls of the hopper is slight so that the calcine flowing through the hopper is practically a thin sheet or layer which, while itself free to pass downward and out of the outlet 23', is fairly gas-proof so that the fumes can 75 not readily escape through it from the fourth into the third hearth. The horizontal or cross-section of the hopper passage-way irrespective of the precise geometric curvature of its opposing walls should conform 80 as much as possible to the curvature of the arc described by the rakes which in their sweep advance the ore along radial lines at substantially uniform speed over the floor of the hearth. The hopper, therefore, if 85 conforming in a measure to the curvature of such arc will be in position to receive its charge in uniform quantities along the full length of the curved slot forming the intake mouth or opening of the hopper passage-way. The doors *D* on the floors *d*, *e*, *f* (and the other floors) are made so as to fit tight, and the space around the shaft where it passes out of the furnace through the bottom plate is made tight by the sand seal 20' 90 (formed by trough 21' and flanged disk 22'). The outlet of the hopper *C* which receives the calcine from the bottom hearth (*f*) is constantly kept sealed by calcine. The bottom hearth is provided with a valve-controlled opening *E* (see valve *V* on the boss *E'*, Fig. 2) for the admission of air to the lower three floors, the hearth *d* being provided with a valve-controlled pipe 24 (see valve *V'* Fig. 2) leading to any suitable 95 exhauster or suction fan *S*, whereby at one operation air is drawn into the chloridizing hearths to facilitate the chloridizing reaction, and the fumes of copper chlorid and acid gases incidental to the reaction are re- 100 105 110 115 120 125 130

5 moved, and may be properly conducted to a suitable absorption tower (not shown). Escape of gases through the openings constituting the hoppers 23, is prevented by 10 maintaining a vacuum on the fourth floor (d) slightly in excess of that (due to draft) on the third floor (c), the small size of the openings especially when charged with ore, preventing mixture by eddy currents. The 15 exhauster coupled to the pipe 24 may of course be operated so as to produce any desired pressure differential between the oxidizing and chloridizing hearths and hence maintain any degree of vacuum in the 20 fourth hearth (d), the pipe 24 leading directly from said hearth. The opening E and the opening for the intake end of the pipe 24 may be positioned of course where most convenient, no definite position being 25 prescribed therefor. By carefully regulating the valves controlling these openings any desired quantity of air may be admitted to, and any desired volume of fumes may be abstracted from, the chloridizing floors; the passage of gases through the openings 30 or hoppers 23 may also be kept at any point desired.

35 The ideal conditions for heating and oxidizing are a thin bed of ore and frequent stirring; the ideal conditions on the other hand for heat conservation and chloridizing are infrequent stirring and a thick bed of ore. Therefore, to maintain these conditions in the oxidizing and chloridizing regions respectively, of the furnace (hearths a, b, c, on the one hand, and hearths d, e, f, on the other hand) two rabble arms (with a proper complement of rakes) per floor are used in the first, second and third hearths, 40 and only one rabble arm per floor is used in the fourth, fifth and sixth hearths, the pitch and spacing of the rakes being properly adjusted to secure the necessary rotary and radial movement of the ore over the floors 45 of the respective hearths (Fig. 4).

50 The principal points of advantage of the present furnace may be summarized as follows:—First. The ore is about two-thirds roasted on the upper three hearths (or floors) and brought up to a good chloridizing heat by direct firing. In this way most of the sulfur is gotten rid of without the consumption of any salt and with a much 55 lower fuel consumption than could be obtained in a muffle-fired furnace. Furthermore since it is not contemplated to complete the roasting in the heated portions of the furnace (hearths a, b, c) there is no need to be over particular about the application 60 of the flame, it being sufficient to pass the ore quickly through a small and rather highly heated region. This gives a greater capacity and greater fuel economy than if a large portion of the furnace (say several 65 floors) were heated moderately. The latter

70 principle is one on which extraneously heated roasting furnaces are generally built, these maintaining the heat by continuous application of heat. In the present furnace the ore is brought rapidly to a roasting temperature after which loss of heat is prevented (in hearths d, e, f), causing the roasting to complete itself in a manner similar to that used for completing the cooking in a “fireless cooker.” Second. The ore when 75 it drops from the third to the fourth floor is in an ideal state for chloridation with a minimum amount of salt, since it has just the correct temperature, and, containing as it does plenty of sulfates to react with the salt, it follows that the chlorin is freely 80 liberated to combine with the metals of the calcine. The volatilization of copper is confined to these (chloridizing) floors and all of this copper can be saved in absorption 85 towers without having to handle the gases from the fire-boxes. The furnace thus possesses the good points of a muffle-furnace as regards the handling of acid and copper fumes. Third. The reasons for combining 90 oxidation and chloridation rather than using either alone are:—a. The first two-thirds 95 say, of the copper is easily oxidized on direct-fired floors with no volatilization of the copper. b. The remaining one-third say, of the copper is oxidized slowly and with difficulty, but rapidly chloridized by the addition of salt. c. Fuel consumption is less for 100 reasons already stated; salt consumption is reduced to a minimum since this is proportional to the sulfur present when salt is added in my furnace, the addition of the salt being made after most of the sulfur has been oxidized. It is true that this furnace 105 will not yield as high a proportion of water-soluble copper as a muffle furnace for sulfating or chloridizing-roasting; but this is of little consequence in a smelting plant treating concentrates, since acid can be 110 made so cheaply that the saving in roasting expense and salt will more than pay for it.

115 The waste gases from the upper three hearths escape through the uptake 25 and pipe 26. The ore traverses the several hearths under the action of the rakes, an operation only too well understood in the art and there is no occasion to repeat it in the present connection.

120 Structural features shown but not alluded to are well known and a description thereof is here unnecessary. Obviously, the number of hearths need not be confined to six, nor need the number of oxidizing hearths necessarily have to correspond to the number of chloridizing hearths. The terms “hearth” 125 and “floor” are here used indiscriminately the two having substantially the same meaning. Where however the floor of a hearth is specifically referred to, such latter expression has reference to the bottom of the 130

hearth in contradistinction to the roof (which forms the floor or bottom of the next hearth above). The opposing walls of the hoppers 23 need not of course be cylindrical; 5 they may be conical or follow the curvature of an ellipse, or the walls of a prism or pyramid or other shape, without departing from the spirit of my invention.

Having described my invention, what I 10 claim is:

1. In combination with a furnace having a series of superimposed intercommunicating hearths, means for subjecting the charge to an oxidizing roast under direct fire in the 15 hearths forming the upper members of the series, the hearths forming the lower members of the series serving as chloridizing hearths, and means for maintaining a pressure differential between the direct-fired 20 hearth and the adjacent chloridizing hearth.

2. In combination with a furnace having a series of superimposed intercommunicating hearths, means for subjecting the charge to an oxidizing roast under direct fire, in 25 the hearths forming the upper members of the series, means for conserving the heat inherent in the charge delivered to the lower hearths whereby the charge may be chloridized in said lower hearths without further 30 application of heat, means for excluding any material passage of fumes from the chloridizing to the oxidizing hearths, and means coupled to the upper member of the chlorid-

izing hearths, for removing the fumes from the chloridizing hearths at a rate sufficient 35 to maintain a pressure differential between the bottom oxidizing hearth, and the adjacent upper chloridizing hearth.

3. In a furnace, a pair of superimposed hearths, rabble mechanism sweeping over 40 the respective hearths from a fixed axis passing through the hearths, hoppers leading from the upper to the lower hearth having narrow passage-ways disposed between 45 curved walls concentric with said axis and conforming substantially with the curvature of the arc defining the sweep of the rabble mechanism.

4. In a furnace, a pair of superimposed hearths, means for advancing the material 50 radially toward the center of the upper hearth, a hopper leading from the upper to the lower hearth and provided with a narrow passage-way having a horizontal curvature concentric with the center toward which 55 the material is advanced, the sides of the hopper tapering downward, and the bottom having a reduced outlet, whereby a sheet of the material fills said hopper while discharging from said reduced outlet. 60

In testimony whereof I affix my signature, in presence of two witnesses.

FREDERICK LAIST.

Witnesses:

ALBERT E. WIGGIN,  
WARREN JENNEY.

Copies of this patent may be obtained for five cents each, by addressing the "Commissioner of Patents,  
Washington, D. C."